# EUROPEAN PATENT SPECIFICATION

(11) **EP 3 597 795 B1**
(45) Date of publication and mention of the grant of the patent: **26.10.2022**
(21) Application number: 19187128.4
(22) Date of filing: 18.07.2019
(51) Int. Cl.: C25D 11/08, C25D 11/10, C25D 11/24

(54) **ANODIZATION METHOD FOR CORROSION PROTECTION OF ALUMINIUM OR ALUMINIUM ALLOY ELEMENTS USED IN AN AIRCRAFT STRUCTURE**
ANODISIERUNGSVERFAHREN ZUM KORROSIONSSCHUTZ VON ALUMINIUM- ODER ALUMINIUMLEGIERUNGSELEMENTEN, DIE IN EINER FLUGZEUGSTRUKTUR VERWENDET WERDEN
PROCÉDÉ D'ANODISATION POUR LA PROTECTION CONTRE LA CORROSION D'ÉLÉMENTS D'ALUMINIUM OU D'ALLIAGE D'ALUMINIUM UTILISÉS DANS UNE STRUCTURE D'AÉRONEF

(30) Priority: 18.07.2018 IT 201800007314
(43) Date of publication of application: 22.01.2020
(73) Proprietor: LEONARDO S.p.A., 00195 Roma (IT)
(72) Inventor: ADDIVINOLA, Bruno, 00195 ROMA (IT); PASTORE, Stefano, 00195 ROMA (IT); ALBOLINO, Augusto, 00195 ROMA (IT); CILIBERTO, Antonio, 00195 ROMA (IT); CUTILLO, Lucia, 00195 ROMA (IT); GALLO, Giuseppe Stefano, 00195 ROMA (IT)
(74) Representative: Bongiovanni, Simone

(56) References cited:
- WO-A1-03/040437
- US-A1- 2006 226 020
- US-A1- 2015 020 925

## Description

### CROSS-REFERENCE TO RELATED APPLICATIONS

This patent application claims priority from Italian patent application no. 102018000007314 filed on July 18, 2018.

### TECHNICAL FIELD

The present invention relates to an anodization method for corrosion protection of aluminium or aluminium alloy elements used in an aircraft structure.

### BACKGROUND OF THE INVENTION

As is known, in order to protect aluminium or aluminium alloy elements used in an aircraft structure, anodization methods have been developed to provide a thin (a few microns) protective layer of metal oxide, which protects the underlying aluminium/aluminium alloy from corrosion. This layer of metal oxide also facilitates the subsequent painting of the aircraft structures and also increases the surface electrical resistance of the aircraft structure.

Typically, the known anodization processes comprise a plurality of steps, including:
a) subjecting the element to a degreasing step by means of an alkaline bath for removing contaminating elements, such as for example oils, fats, lubricants, protective layers, dusts and residues in general - then subjecting it to a first washing in water;
b) subjecting the element to an acid pickling step. Then extracting the element from the acid solution and subjecting the element to a subsequent washing in water. This step contributes to the removal of natural oxide, thermal oxides, traces of materials deposited as a result of mechanical processing, scratches, discolourations, mild corrosion;
c) subjecting the washed element to a subsequent electrochemical treatment step by dipping the element in a chromic acid solution (using chromium with an oxidation number of +6 - hexavalent chromium) and applying an electric potential to this element;
d) subjecting the element to a subsequent second washing in water;
e) dipping the element in a bath in which a solution of a chromium compound with an oxidation number of +6 (hexavalent chromium) is present, in order to carry out a post-anodization sealing step;
f) extracting the element from the bath of step e) and subjecting it to a third final washing.

This method uses very dangerous compounds, such as H₂CrO₄, commonly called chromic acid where the chromium has an oxidation number of +6; it is a highly oxidizing species. The chemical reaction that occurs is the following: Electrochemical reaction at the anode:

**2Al + 3H₂O = Al₂O₃ + 6H⁺ + 6e⁻**

Electrochemical reaction at the cathode:

**6H⁺ + 6e⁻ = 3H₂**

Resulting anodization reaction:

**2Al + 3H₂O => Al₂O₃ + 3H₂**

Aluminium chromate will also be formed according to the following mechanism:

chromic anhydride -> chromic acid -> aluminium chromate CrO₃ -> H₂CrO₄ -> Al₂(CrO₄)₃

Furthermore, on the basis of experimental and epidemiological evidence, chromium with an oxidation number of +6 (hexavalent chromium) has been classified by IARC as a human carcinogen (Class I).

With regard to the effects on health, several studies have demonstrated that exposure to hexavalent chromium is one of the possible causes of lung cancer, as it is mutagenic and carcinogenic. In fact, the respiratory system is the main target of the toxic and carcinogenic action, and acute and chronic occupational exposure occurs above all by absorption through inhalation. The toxicity of the hexavalent form at the intracellular level appears above all with the numerous molecular and structural alterations caused by the unstable [Cr(V) and Cr(IV)] and stable [Cr(III)] forms resulting from the reduction process.

US2015020925 describes a method for the surface treatment of an aluminum, magnesium or one of its alloys, to protect the part from corrosion. The method consists in consecutively immersing the part in the following two baths:
- first aqueous bath at low temperatures containing a corrosion inhibiting metal salt and an oxidizing compound to form a conversion coating on the surface of the part containing oxides, hydroxides and fluorides based on Zirconium / Chromium;
- a second aqueous bath, kept at a temperature below 80 ° C and containing an oxidizing compound and a rare earth salt corrosion inhibitor. Through the presence of hydrogen peroxide, the oxidation of chromium is obtained from the trivalent to the hexavalent form and the formation of chromates.

The method can be performed for the chemical conversion of aluminum or its alloys and magnesium or its alloys, on parts that have not been previously treated or after anodizing the piece to seal the anodic layer.

US2015020925 describes alkaline degreasing, subsequent acid pickling and an anodizing step of a metal part with a bath comprising sulphuric acid and tartaric acid. At the end of an anodizing step a sealing step is performed on the metal part using a solution of trivalent chromium and zirconium.

WO03040437A1 discloses a post anodization treatment wherein it is used an acidic aqueous solution having a pH ranging from about 2.5 to 4.5 and containing trivalent chromium salts, alkali metal hexafluorozirconates, an alkali metal fluoro-compound e.g. fluoroborates and/or fluorosilicates.

Therefore, there is a need to develop a method which does not use toxic/carcinogenic materials and allows the formation of an oxide layer that provides good protection to the underlying aluminium/aluminium alloy.

### SUMMARY OF THE INVENTION

The above object is achieved by the present invention in so far as it relates to an anodization method for corrosion protection of an aluminium or aluminium alloy element used in an aircraft structure, **comprising** the following steps:
a) subjecting the element to a degreasing step by means of an alkaline bath (block 100) for removing contaminating elements;
b) subjecting the element to a subsequent first washing in water (block 110);
c) subjecting the element to an acid pickling step (120) by dipping the element in an acid solution and then extracting the element from the acid solution and subjecting the element to a subsequent washing in water;
d) subjecting the washed element to a subsequent electrochemical treatment step in a tank (140) by dipping the element in a solution of tartaric acid (C₄H₆O₆) and sulphuric acid (H₂SO₄) and applying an electric potential to said element;
e) subjecting the element to a subsequent second washing in water (150);
f) dipping (block 170) the element in a bath in which a solution of chromium, with an oxidation number of +3, and zirconium ions and fluorides is present, in order to carry out a post-anodization sealing step;
g) extracting the element from the bath of step f) and subjecting it to a third final washing in water and a subsequent dipping in a tank of boiling water, which provides a second sealing step, and then drying the element (block 180) .

### BRIEF DESCRIPTION OF THE DRAWINGS

The invention will now be illustrated with reference to the accompanying figures wherein:
Figure 1 represents a non-limiting embodiment showing the main steps of the method according to the present invention; and
Figure 2 specifies one step of the method of the present invention.

### DETAILED DESCRIPTION OF THE INVENTION

With reference to Figure 1, the anodization method for corrosion protection of an aluminium or aluminium alloy element used in an aircraft structure **comprises** the following steps:
a) subjecting the element to a degreasing step by means of an alkaline bath (block 100) for removing contaminating elements, such as for example oils, fats, lubricants, protective layers, dusts and residues in general. Typically, step a) is carried out by dipping the element in the alkaline bath for a time interval of 10 - 20 minutes. Typically, the alkaline bath has a temperature of approximately 55 ± 5 degrees Celsius.
b) subjecting the element to a subsequent first washing in water (block 110). Typically, step b) is carried out with water for a time ranging from 2 to 5 minutes at a temperature below 35 degrees Celsius.
c) subjecting the element to an acid pickling step (block 120) by dipping the element for approximately 5-10 minutes in an acidic solution based on ferric sulphate and a mixture of acids maintained at a temperature comprised between 20°C and 40°C and then extracting the element from the acidic solution and subjecting the element to a subsequent washing in water (block 130 following block 120) for 4 - 10 minutes at room temperature and assessing the film of water. Checking by assessing the film of water on the surface of the part during the rinsing ensures the effectiveness of the pretreatment. Step c) contributes to the removal of natural oxide, thermal oxides, traces of materials deposited as a result of mechanical processing, scratches, discolourations, mild corrosion;
d) subjecting the washed element to a subsequent electrochemical treatment step in a tank (block 140) by dipping the element in a solution of tartaric acid (C₄H₆O₆) and sulphuric acid (H₂SO₄) and applying an electric potential, wherein the aluminium/aluminium alloy element behaves as the anode (positive pole) whereas the negative electrode (or cathode) is represented by the tank. Step d) is carried out with a solution having a temperature comprised between 36 and 39 degrees Celsius. The typical concentration of tartaric acid is 72-88 g/l and that of sulphuric acid is 36-44 g/l.

The chemical reaction occurring in step d) is the following:
Electrochemical reaction at the anode:

   **2Al + 3H₂O = Al₂O₃ + 6H⁺ + 6e⁻**
Electrochemical reaction at the cathode:

   **6H⁺ + 6e⁻ = 3H₂**
Resulting anodization reaction:

   **2Al + 3H₂O => Al₂O₃ + 3H₂**
Aluminium sulphate, which contributes to the protection of the underlying metal/metal alloy, will also be formed according to the following mechanism:

   **3H₂SO₄ + 2Al ←→ Al₂(SO₄)₃ + 3H₂**

Step d) is typically performed using the following parameters (see Figure 2):
- applying on the element the voltage within one minute from the dipping of the element in the solution;
- subsequently and without interruption applying on the element an increasing voltage with a ramp not exceeding 3 volts per minute;
- subsequently and without interruption applying on the element a constant voltage (approximately 14 Volts) for approximately 20 minutes, and thereafter;
- gradually reducing the applied voltage to a null value in approximately one minute;
- removing the element from the solution within 3 minutes from the switching off of the voltage

e) subjecting the element to a subsequent second washing in water (block 150). Typically, step e) **comprises** an optional rinsing step by dipping in industrial water (block 150a) at room temperature and a subsequent rinsing step by dipping in purified water at room temperature (block 150b). Subsequently, the washed element is subjected to visual inspection by an operator (block 160) and, if this step is fulfilled, the following step is carried out:
f) dipping (block 170) the element in a bath in which chromium, with an oxidation number of +3, zirconium ions and fluorides (resulting from salts and fluorozirconates/silicates) are present, in order to carry out a first post-anodization sealing step;
The chemical reaction that occurs is the following:

   **4Al2O3 + 24F⁻ + 3Zr⁺⁴ + 4Cr⁺³ → 8AlF3 + 3ZrO2 + 2Cr2O3**

Typically, the dipping time in step f) is comprised between 2 and 20 minutes. It is suggested a time comprised between 2 and 3 minutes.

g) extracting the element from the bath of step f) and subjecting it to a third final washing and a subsequent dipping in a tank of boiling water (temperature comprised between 95 and 100 degrees Celsius, pH ranging from 4.5 to 7, for approximately 30 minutes), which provides a second sealing step, according to the following reaction:

**Al₂O₃ + H₂O -> 2 AlO (OH) (an aluminium oxide hydroxide-böhmite)**

Which results in a volume increase, which is responsible for the "filling" of the pores of the anodic oxide. The reduction in porosity resulting from alumina hydration drastically reduces the adsorption capacity, making the surface insensitive to fingerprints, colour and grease stains, and giving the oxide a greater resistance to corrosion. To achieve the above reaction and to obtain A10 (OH) (aluminum hydroxide oxide), the temperature has a fundamental influence. If in fact the temperature were lower than the one highlighted above, a layer of aluminum hydroxide [Al (OH) 3] would be created with different characteristics and with a percentage of hydration of the oxide that would not guarantee the same resistance to corrosion.

Drying the element (block 180). Typically, the drying can be carried out in a dust-free environment, for example an oven that reaches a temperature between 45 and 65 degrees Celsius for at least 20 minutes.

Between step b) and step d) the following further steps may also be carried out, optional to step c), which is carried out anyway:
rapid alkaline chemical etching (block 200) with a caustic soda based solution in order to prepare/activate the aluminium/aluminium alloy surfaces for the electrochemical treatment in step d). Typically, this step is carried out by dipping the element in an alkaline solution having a temperature of approximately 60 degrees for 30-60 seconds; and
Aluminium desmutting and rinsing (block 210). Typically, this step of clearing the blackening due to the preceding alkaline bath is performed by dipping the element in a clearing solution (based on ferric sulphate and a mixture of acids) at room temperature (approximately 25 degrees) for 5-10 minutes.

From the above description it appears that the method of the present invention, in particular the sealing (step f), does not use highly toxic, and in particular carcinogenic compounds, such as chromium with an oxidation number of +6. The sealed oxide layer has a sensibly constant thickness of a few microns (typically from 2 to 7 microns) and good adhesion characteristics. The elements are therefore effectively protected from corrosion.

The Applicant performed a series of mechanical fatigue tests on samples subjected to the method of the present invention. The tests were carried out on cylindrical specimens treated according to the method of the present invention in accordance with standard EN6072 provided in the aeronautical field. Results were plotted in a Wohler curve at various load levels.

By comparing the data, the treatment according to the present method was thus shown not to alter the fatigue resistance of the sample, which complies with the CS 25.571 aeronautical directives. Corrosion tests, which were carried out in a salt spray chamber for ASTM B 117, also performed well. In this case, a salt spray chamber was used, which was capable of providing a controlled saline environment fed by a 5% NaCl salt solution. Tests for permanence in the salt spray for 336 hours were brilliantly passed.

Tests for adhesion of the paint to the elements treated according to the method of the present invention were also carried out. These tests were carried out in accordance with ISO 2409 standard after dipping in demineralized water at 23 degrees Celsius for 14 days. The test consists in squaring off, after the dipping in water, the paint layer with a six-blade cutter, arranging and pressing a layer of tape against the squared paint and then tearing off the tape quickly. The tests gave a positive result, with a detachment of the coating paint of less than 5%.

## Claims

1. An anodization method for corrosion protection of an aluminium or aluminium alloy element used in an aircraft structure, **comprising** the following steps:
a) subjecting the element to a degreasing step by means of an alkaline bath (100) for removing contaminating elements;
b) subjecting the element to a subsequent first washing in water (110);
c) subjecting the element to an acid pickling step (120) by dipping the element in an acid solution and then extracting the element from the acid solution and subjecting the element to a subsequent washing in water;
d) subjecting the washed element to a subsequent anodization step in a tank (140) by dipping the element in a solution of tartaric acid (C₄H₆O₆) and sulphuric acid (H₂SO₄) and applying an electric potential to said element that acts as anode;
e) subjecting the element to a subsequent second washing in water (150);
f) dipping ( 170) the element in a bath in which a solution of chromium, with an oxidation number of +3, and zirconium ions and fluorides is present, in order to carry out a post-anodization sealing step;
g) extracting the element from the bath of step f) and subjecting it to a third final washing in water and a subsequent dipping in a tank of water having a temperature comprised between 95° and 100°, which provides a second sealing step, and then drying the element (180).

2. The anodization method as defined in claim 1, wherein step c) is carried out by dipping the element in an acid bath for a time interval of 5 to 10 minutes.

3. The anodization method as defined in claim 1 or 2, wherein step c) is carried out by dipping the element in an acid bath having a temperature of 20°C to 40°C.

4. The anodization method as defined in any one of the preceding claims, wherein step d) is configured to perform the following chemical reactions:
Electrochemical reaction at the anode:
**2Al + 3H₂O = Al₂O₃ + 6H⁺ + 6e⁻**
Electrochemical reaction at the cathode:
**6H⁺ + 6e⁻ = 3H₂**
Resulting anodization reaction:
**2Al + 3H₂O => Al₂O₃ + 3H₂**

5. The anodization method as defined in any one of the preceding claims, wherein step d) is carried out using the following parameters:
applying to the element the voltage within one minute from the dipping of the element in the solution;
subsequently applying to the element an increasing voltage with a ramp not exceeding 3 volts per minute;
subsequently and without interruption applying to the element a constant voltage for approximately 20 minutes, and thereafter;
subsequently gradually reducing the applied voltage to a null value;
finally removing the element from the solution within 3 minutes from the switching off of the voltage.

6. The anodization method as defined in any one of the preceding claims, wherein step d) is carried out using a solution having a temperature ranging between 36°C and 39°C.

7. The anodization method as defined in any one of the preceding claims, wherein step g) is carried out in a tank of boiling water with a temperature higher than 95°C and a pH ranging between 4.5 and 7 for approximately 30 minutes.

8. The anodization method as defined in any one of the preceding claims, wherein in step d) the concentration of tartaric acid is 72-88 g/l and the concentration of sulphuric acid is 36-44 g/l.

9. The anodization method as defined in any one of the preceding claims, wherein step f) performs the following chemical reactions:
**4Al2O3 + 24F⁻ + 3Zr⁺⁴ + 4Cr⁺³ → 8AlF3 + 3ZrO2 + 2Cr2O3**

10. The anodization method as defined in any one of the preceding claims, wherein between step b) and step d) the following further steps are also carried out:
alkaline chemical etching (200) in order to prepare/activate the aluminium/aluminium alloy surfaces for the electrochemical treatment in step d); and
aluminium/aluminium alloy desmutting and rinsing (210).

11. The anodization method as defined in any one of the preceding claims, wherein said boiling water has a pH ranging between 4.5 and 7.

12. The anodization method as defined in any one of the preceding claims, wherein said fluorides result from salts and fluorozirconates/silicates.

## Patentansprüche

1. Eloxierungsverfahren zum Korrosionsschutz eines Aluminium- oder Aluminiumlegierungselements, das in einer Luftfahrzeugstruktur verwendet wird, das die folgenden Schritte umfasst:
a) Unterwerfen des Elements einem Entfettungsschritt mittels eines Alkalibads (100) zum Entfernen von verunreinigenden Elementen;
b) Unterwerfen des Elements einem nachfolgenden ersten Waschen in Wasser (110);
c) Unterwerfen des Elements einem Säurebeizschritt (120) durch Tauchen des Elements in einer Säurelösung und dann Entnehmen des Elements aus der Säurelösung und Unterwerfen des Elements einem nachfolgenden Waschen in Wasser;
d) Unterwerfen des gewaschenen Elements einem nachfolgenden Eloxierungsschritt in einem Behälter (140) durch Tauchen des Elements in eine Lösung aus Weinsäure (C₄H₆O₆) und Schwefelsäure (H₂SO₄) und Anlegen eines elektrischen Potentials an das Element, das als Anode wirkt;
e) Unterwerfen des Elements einem nachfolgenden zweiten Waschen in Wasser (150);
f) Tauchen (170) des Elements in ein Bad, in dem eine Lösung von Chrom mit einer Oxidationszahl von +3 und Zirkonionen und Fluoriden vorhanden ist, um einen Nacheloxierungsversiegelungsschritt auszuführen; und
g) Entnehmen des Elements aus dem Bad von Schritt f) und Unterwerfen des Elements einem dritten endgültigen Waschen in Wasser und einem nachfolgenden Tauchen in einen Behälter von Wasser, das eine Temperatur besitzt, die im Bereich von 95° bis 100° liegt, was einen zweiten Versiegelungsschritt bereitstellt, und dann Trocknen des Elements (180).

2. Eloxierungsverfahren nach Anspruch 1, wobei Schritt c) durch Tauchen des Elements in ein Säurebad für ein Zeitintervall im Bereich von 5 bis 10 Minuten ausgeführt wird.

3. Eloxierungsverfahren nach Anspruch 1 oder 2, wobei Schritt c) durch Tauchen des Elements in ein Säurebad, das eine Temperatur im Bereich von 20 °C bis 40 °C besitzt, ausgeführt wird.

4. Eloxierungsverfahren nach einem der vorhergehenden Ansprüche, wobei Schritt d) konfiguriert ist, die folgenden chemischen Reaktionen durchzuführen:
Elektrochemische Reaktion bei der Anode:
2Al + 3H₂O = Al₂O₃ + 6H⁺ + 6e⁻
Elektrochemische Reaktion bei der Kathode:
6H⁺ + 6e⁻ = 3H₂
Resultierende Eloxierungsreaktion:
2Al + 3H₂O => Al₂O₃ + 3H₂

5. Eloxierungsverfahren nach einem der vorhergehenden Ansprüche, wobei Schritt d) unter Verwendung der folgenden Parameter ausgeführt wird:
Anlegen an das Element der Spannung in einer Minute vor dem Tauchen des Elements in die Lösung;
anschließend Anlegen an das Element einer zunehmenden Spannung mit einem Anstieg, der 3 Volt pro Minute nicht überschreitet;
anschließend und ohne Unterbrechung Anlegen an das Element einer konstanten Spannung für etwa 20 Minuten und danach;
anschließend allmähliches Verringern der angelegten Spannung zu einem Nullwert und
schließlich Entfernen des Elements aus der Lösung in 3 Minuten ab dem Abschalten der Spannung.

6. Eloxierungsverfahren nach einem der vorhergehenden Ansprüche, wobei Schritt d) unter Verwendung einer Lösung ausgeführt wird, die eine Temperatur besitzt, die im Bereich von 36 °C bis 39 °C liegt.

7. Eloxierungsverfahren nach einem der vorhergehenden Ansprüche, wobei Schritt g) in einem Behälter kochenden Wassers mit einer Temperatur größer als 95 °C und einem pH-Wert, der zwischen 4,5 und 7 liegt, für etwa 30 Minuten ausgeführt wird.

8. Eloxierungsverfahren nach einem der vorhergehenden Ansprüche, wobei in Schritt d) die Konzentration von Weinsäure 72-88 g/l ist und die Konzentration von Schwefelsäure 36-44 g/l ist.

9. Eloxierungsverfahren nach einem der vorhergehenden Ansprüche, wobei Schritt f) die folgenden chemischen Reaktionen durchführt:
4Al2O3 + 24F⁻ + 3Zr⁺⁴ + 4Cr⁺³ → 8AlF3 + 3Zr02 + 2Cr203

10. Eloxierungsverfahren nach einem der vorhergehenden Ansprüche, wobei zwischen Schritt b) und Schritt d) außerdem die folgenden weiteren Schritte ausgeführt werden:
basisches chemisches Ätzen (200), um die Aluminium-/Aluminiumlegierungsoberflächen für die elektrochemische Behandlung in Schritt d) vorzubereiten/zu aktivieren; und
Belagentfernung und Spülen (210) des Aluminiums/der Aluminiumlegierung.

11. Eloxierungsverfahren nach einem der vorhergehenden Ansprüche, wobei das kochende Wasser einen pH-Wert besitzt, der zwischen 4,5 und 7 liegt.

12. Eloxierungsverfahren nach einem der vorhergehenden Ansprüche, wobei die Fluoride aus Salzen und Flurozirkonaten/Silicaten resultieren.

## Revendications

1. Méthode d'anodisation pour la protection contre la corrosion d'un élément en aluminium ou en alliage d'aluminium utilisé dans une structure d'aéronef, comprenant les étapes suivantes :
a) la soumission de l'élément à une étape de dégraissage au moyen d'un bain alcalin (100) pour retirer les éléments contaminants ;
b) la soumission de l'élément à un premier lavage ultérieur à l'eau (110) ;
c) la soumission de l'élément à une étape de décapage acide (120) en trempant l'élément dans une solution acide puis en extrayant l'élément de la solution acide et la soumission de l'élément à un lavage ultérieur à l'eau ;
d) la soumission de l'élément lavé à une étape d'anodisation ultérieure dans une cuve (140) en trempant l'élément dans une solution d'acide tartrique (C₄H₆O₆) et d'acide sulfurique (H₂SO₄) et en appliquant un potentiel électrique audit élément qui agit comme anode ;
e) la soumission de l'élément à un deuxième lavage ultérieur à l'eau (150) ;
f) le trempage (170) de l'élément dans un bain contenant une solution de chrome, d'indice d'oxydation +3, et d'ions de zirconium et de fluorures, pour réaliser une étape de scellement post-anodisation ;
g) l'extraction de l'élément du bain de l'étape f) et sa soumission à un troisième lavage final à l'eau et à un trempage ultérieur dans un réservoir d'eau ayant une température comprise entre 95° et 100°, ce qui fournit une deuxième étape de scellement, puis séchage de l'élément (180).

2. Méthode d'anodisation selon la revendication 1, dans laquelle l'étape c) est réalisée en trempant l'élément dans un bain acide pendant un intervalle de temps de 5 à 10 minutes.

3. Méthode d'anodisation selon la revendication 1 ou 2, dans laquelle l'étape c) est réalisée en trempant l'élément dans un bain acide ayant une température de 20 °C à 40 °C.

4. Méthode d'anodisation selon l'une quelconque des revendications précédentes, dans laquelle l'étape d) est configurée pour effectuer les réactions chimiques suivantes :
réaction électrochimique à l'anode :
**2Al + 3H₂O = Al₂O₃ + 6H⁺ + 6e⁻**
réaction électrochimique à la cathode :
**6H⁺ + 6e⁻ = 3H₂**
réaction d'anodisation résultante :
**2Al + 3H₂O => Al₂O₃ +** 3H₂

5. Méthode d'anodisation selon l'une quelconque des revendications précédentes, dans laquelle l'étape d) est réalisée en utilisant les paramètres suivants :
l'application à l'élément de la tension dans la minute qui suit le trempage de l'élément dans la solution ;
l'application ultérieure à l'élément d'une tension croissante avec une rampe n'excédant pas 3 volts par minute ;
l'application ultérieure et sans interruption à l'élément d'une tension constante pendant environ 20 minutes, et par la suite ;
la réduction progressive ultérieure de la tension appliquée jusqu'à une valeur nulle ;
enfin, le retrait de l'élément de la solution dans les 3 minutes qui suivent la coupure de la tension.

6. Méthode d'anodisation selon l'une quelconque des revendications précédentes, dans laquelle l'étape d) est réalisée en utilisant une solution ayant une température dans la plage entre 36 °C et 39 °C.

7. Méthode d'anodisation selon l'une quelconque des revendications précédentes, dans laquelle l'étape g) est réalisée dans un réservoir d'eau bouillante à une température supérieure à 95°C et un pH dans la plage entre 4,5 et 7 pendant environ 30 minutes.

8. Méthode d'anodisation selon l'une quelconque des revendications précédentes, dans laquelle à l'étape d) la concentration en acide tartrique est de 72 à 88 g/l et la concentration en acide sulfurique est de 36 à 44 g/l.

9. Méthode d'anodisation selon l'une quelconque des revendications précédentes, dans laquelle l'étape f) effectue les réactions chimiques suivantes :
**4Al2O3 + 24F⁻ + 3Zr⁺⁴ + 4Cr⁺³ → 8AlF3 + 3ZrO2 + 2Cr2O3**

10. Méthode d'anodisation selon l'une quelconque des revendications précédentes, dans laquelle entre l'étape b) et l'étape d) les étapes supplémentaires suivantes sont également réalisées :
attaque chimique alcaline (200) afin de préparer/activer les surfaces d'aluminium/d'alliage d'aluminium pour le traitement électrochimique à l'étape d) ; et
décapage et rinçage (210) de l'aluminium/de l'alliage d'aluminium.

11. Méthode d'anodisation selon l'une quelconque des revendications précédentes, dans laquelle ladite eau bouillante a un pH dans la plage entre 4,5 et 7.

12. Méthode d'anodisation selon l'une quelconque des revendications précédentes, dans laquelle lesdits fluorures sont issus de sels et de fluorozirconates/silicates.
